

Sept. 17, 1935.

D. K. ALLISON

2,014,606

THREE-COLOR FILM AND PROCESS

Filed May 12, 1934

Fig. 1.



Fig. 2.



Fig. 3.

MATRIX PROCEDURE A.



MATRIX PROCEDURE B.



INVENTOR.  
DONALD K. ALLISON  
BY *Robert M. Fulwiler*  
ATTORNEYS.

## UNITED STATES PATENT OFFICE

2,014,606

## THREE-COLOR FILM AND PROCESS

Donald K. Allison, Beverly Hills, Calif.

Application May 12, 1934, Serial No. 725,311

6 Claims. (Cl. 95—2)

This invention relates in general to color photography and finds its most valuable application in the field of motion picture production, although it may be applied with equally effective results to still photography. Whenever the term film is used, it is to be understood that it comprehends all types thereof, including plates, film for still work, film for motion picture work and all other types of photographic media. However, inasmuch as my invention finds its chief application in cinematography, I will illustrate a preferred and modified form thereof in this connection without however, limiting myself thereto.

15 Numerous processes have been evolved for the making of motion pictures in color and they have more or less divided themselves into two main classes known as additive and subtractive. The production of negatives by subtractive processes 20 has in turn been divided into the multi-pack system, the commonly known being bi-pack, and the light-splitting or separating method. As to the production of positive prints, it has been divided into photographic printing and photomechanical or imbibition printing, depending on how the positives are produced from the color separation negatives.

25 For the production of negatives, my invention preferably employs the bi-pack system because of its simplicity and economy of operation, although the light splitting or separating system can be used, just so long as accurate color separation is obtained. In the production of positives by my process, I utilize in the preferred forms thereof both photographic and photomechanical printing to secure a three-color positive from but two original negatives.

30 It has long been the aim of all research workers in the field of color photography to produce accurate three-color rendition by using but two negatives, and it is an object of my invention to produce such three-color rendition in positive prints by the use of but two negatives. So far as I am aware, this has never before been accomplished satisfactorily.

35 It is also an object of my invention to provide a color process that will attain this result accurately, while being at the same time relatively simple and economical in operation and positive in its reproduction of colors.

40 Another object of my invention is to provide a three-color process that can be readily adapted to existing two-color processes so that by a comparatively slight modification of existing two-

color laboratories, they can be made capable of producing satisfactory three-color prints. A further advantage being that no change in cameras or photographing technique is needed to accompany such a plant change-over.

5 Other objects and advantages of my film and method of making the same will become apparent from the following description of a preferred form and modification thereof.

In the attached drawing:

10 Fig. 1 shows a preferred form of positive film being printed photographically from two color-separation negatives.

Fig. 2 shows a modified form of positive film being printed.

15 Fig. 3 is a chart showing the steps of preferred form of the entire process and two different procedures for securing the matrix.

20 As previously mentioned, I prefer to use the bi-pack system of securing color separation negatives, which system consists briefly in running two films through the camera gate face to face. The outside negative or the one on which the light first impinges may be of the type usually designated in the trade as orthochromatic, and is sensitive to substantially the blue to green range of the spectrum only. I will term this negative hereafter the "front" or "ortho" negative. After the light impinges on the front negative, it passes therethrough onto the second or rear negative 25 which is known as a panchromatic film and is sensitive to substantially all colors but predominantly to the orange to red end of the spectrum. This negative I will hereafter speak of as the "rear" or "pan" negative.

30 Due to the fact that the rear negative is sensitive to all colors, it is necessary to filter out all blue light passing through the front negative before it strikes the rear negative. This can be readily accomplished by dyeing the front negative 40 with a substantially orange-red surface dye such as diphenyl-disazo-bis-a-naphthyl-amine-4-sulphonic acid, known generally as Congo red or the like which will allow a slight amount of green and the yellow and red rays to reach the 45 rear film. Bi-pack film of this general type with a red filter dye in the ortho negative is readily available on the market under various trade names.

50 After exposure of the two negatives they are developed and fixed by any of the well-known methods and the red filter dye washed out of the front negative. From the foregoing it will be evident that the front negative carries a silver image recording the blue to green colors of the objects 55

photographed and the rear negative carries a silver image of the green to red colors of the objects, it being noted that the green is recorded on both front and rear negatives.

5 Various processes are now known and commercially available for producing two-color positive prints from such color value negatives, one of the simplest and most effective being to photographically print the two negatives in registry 10 to opposite sides of a double-coated positive film and then tone, dye, or dyetone the side of the positive printed from the ortho negative red, and then tone, dye, or dyetone the side of the positive 15 printed from the pan negative blue. This gives a very satisfactory product for two color rendition, but, of course, using but two primary colors the full range of the spectrum cannot be reproduced.

In using my invention, I may produce a two color positive print such as the one just described, 20 it being possible to use any one of a number of processes, as for example the one wherein the side to be colored blue is treated with an iron tone to convert the images on that side to a blue iron salt, and then the film is immersed in a uranium toning solution to convert the images on the other 25 side to a red uranium salt. Suitable formulas for these solutions are:

Blue tone

|    |                         |           |
|----|-------------------------|-----------|
| 30 | Ferric ammonium oxalate | 9 grams   |
|    | Potassium ferricyanide  | 5 grams   |
|    | Ammonium chloride       | 11 grams  |
|    | Hydrochloric acid       | 6 c.c.    |
|    | Water                   | 1000 c.c. |

35 Uranium tone

|    |                        |           |
|----|------------------------|-----------|
|    | Uranium nitrate        | 9 grams   |
|    | Potassium oxalate      | 6 grams   |
|    | Potassium ferricyanide | 7 grams   |
|    | Hydrochloric acid      | 8 c.c.    |
| 40 | Water                  | 1000 c.c. |

If desired, I can produce the two color positive by employing what is known in the art as the 45 iodide bleach process by which method one side of the film to be colored is first bleached with a solution such as:

|    |                  |           |
|----|------------------|-----------|
| 45 | Iodine           | 15 grams  |
|    | Potassium iodide | 60 grams  |
|    | Acetic acid      | 25 c.c.   |
| 50 | Water            | 1000 c.c. |

55 and then subjected to a basic red or blue dye, depending on which side is treated, which said dye is mordanted on the iodide image. The other side of the film can then be treated in a similar manner or can be toned with iron or uranium as previously explained to secure a blue or a red image as needed. Likewise a copper toning solution can be used for coloring the red side of the film which 60 can be amplified, if desired, by an additional treatment with a basic red dye which is mordanted by the copper image. A suitable copper tone and mordant is:

|    |                        |           |
|----|------------------------|-----------|
| 55 | Cupric sulphate        | 20 grams  |
|    | Potassium ferricyanide | 15 grams  |
|    | Potassium citrate      | 120 grams |
|    | Ammonium carbonate     | 10 grams  |
|    | Water                  | 1000 c.c. |

70 There are, of course, numberless methods of producing a two color positive by photographic printing and subsequent toning, dyeing or dyetoning, each with its proponents and each having certain advantages. The particular method of accomplishing this first step of my process 75 forms no part of my invention except that it shall

be one which will give sufficiently transparent images for commercial projection use.

After I have produced my two color-separation negatives and a two-color positive print therefrom by any suitable method as just explained, I 5 prefer to proceed in one of two ways to build up my two-color print into a three-color one. In that one of these preferred procedures is more simple to perform than the other, I will refer to it as procedure A, describing it first, although it will 10 be understood that the second procedure, referred to herein as procedure B, while being a little longer, gives the better results.

In carrying out procedure A, I produce a matrix from the ortho negative by making a duplicate or "dupe" of the ortho negative by making 15 a print therefrom on ordinary positive duping stock, producing what is termed a lavender or duping print, and then making a print from the lavender print which will, of course, be a negative 20 of the object photographed.

I then treat the dupe negative with an etching solution which can be made up substantially as follows:

|                        |      |       |    |
|------------------------|------|-------|----|
| Hydrogen peroxide (3%) | 30   | c.c.  | 25 |
| Cupric sulphate        | 20   | grams |    |
| Nitric acid (conc.)    | 5    | c.c.  |    |
| Potassium bromide      | 0.5  | grams |    |
| Water                  | 1000 | c.c.  | 30 |

The effect of this solution on the film is to entirely remove the silver image and the gelatin contiguous to the silver image, leaving a gelatin relief image which is the reverse of the silver image of the object photographed. In this case 35 it will be remembered that my ortho negative recorded only the blue and a portion of the green of the objects, and consequently the gelatin relief image obtained by etching the ortho gives us a relief image recording the yellows and reds, 40 and a portion of the greens.

Using the relief image film as a matrix, a yellow, preferably acid, dye is impregnated into the gelatin of this matrix, and from this a yellow image is then imbibed or photomechanically 45 printed in registry on one side of the two color print already obtained. In practice I have found it preferable to imbibe the yellow image on the red side of the two-color print, although it can be imbibed on the blue side of the print, if desired.

The effect of imbibing the third color, yellow, onto the two-color print is to give us full range 55 reproduction of the visible spectrum. While the yellow dye is actually applied to the yellow, orange and red images, the effective result is that the portion which is represented yellow, comes out yellow for the density of the image being low, the amount of red coloring is small, so that the yellow dye imbibed thereon predominates and blocks out the red. As to the orange which is a little heavier density than the yellow, the only effect of imbibing a yellow dye thereon is to brighten it up and make it a truer orange. The full red portion of the image which is the 60 heaviest density is not affected appreciably by the application of the yellow dye. The result then is that we have yellows, oranges and reds 65 faithfully reproduced on the side of the positive printed from the ortho negative and previously 70 colored red.

As before mentioned, the greens are recorded on both front and rear negatives and it was noted that in printing, the greens were therefore 75 printed on each side of the positive, and at the

end of the first step of my process were formed of a thin blue image on one side of the print and a very thin orange image on the opposite side thereof in registry with the blue image. As my 5 matrix formed from the dupe ortho negative records greens to a slight extent, it will, of course, imbibe yellow dye on that portion of the light orange colored positive which is supposed to be green and then the resultant yellow image in 10 combination with the blue will reproduce a true green when projected on the screen.

In practicing my second or alternative method, I produce a matrix from the pan negative for 15 imbibing the yellow image. This method, which I term procedure B, is as follows:

The pan negative is printed onto ordinary black and white positive stock and then without developing up the latent image thus obtained, the uncolored print previously made by printing 20 in registry to opposite sides of a double-coated positive, is used to superpose a print on the undeveloped print made from the pan negative. The superposed latent images are then developed up and fixed in the usual manner.

The composite print thus obtained is then 25 reverse etched by treatment with a suitable solution such as the one previously mentioned, to produce a matrix composed of a gelatin relief image substantially similar to the matrix formed 30 by the first method described. There is, however, one essential difference and advantage of this second matrix over the one made from the ortho negative, namely that in this second form of matrix only the greens, yellows and reds are 35 in relief, the blues, grays, whites and blacks being washed out, whereas in the first matrix the grays and blacks are also in relief as well as the greens, yellows and reds. I have found that in the process first described, imbibing yellow on the blacks 40 does not appreciably affect them, i. e., black by this process is made from red and blue, with an allowance for the addition of yellow. However, in the case of the grays the addition of the yellow is sometimes noticeable and has a slight tendency to give them a muddy effect.

The color balance maintained between the red and the blue will, of course, depend on which type of matrix is employed, for if type A is used, blacks are the subtractive result of blue, red 50 and yellow, whereas, if type B matrix is used, blacks are the subtractive result of red and blue only.

While I have deemed it necessary to describe 55 in detail only two methods or procedures for producing a suitable matrix for use in my process, it is to be understood that I do not limit myself to these two forms shown, as my invention in its broad aspect comprehends a three-color print formed by the addition of a third image by imbibing from any suitable matrix obtained by the use of one or both of two color-separation negatives, on to a two-color print previously produced from said two color-separation negatives. There are various other known methods of preparing matrices which are eminently satisfactory 60 for this work. Some of these methods are for example, the bichromate process, in which the gelatin carrying a silver image, when treated with bichromate, becomes insoluble in hot water in the image areas; the pinatype process in which bichromated colloid, usually gelatin, becomes insoluble in hot water in areas exposed to light; and the developed relief processes, in which 65 the end-products of the developing reactions

cause insolubilization of the gelatin contiguous to the image.

I cite these various methods of making matrices to show the wide range of operations by which my invention may be practiced. It should 5 be noted, however, that the above lastly described relief processes yield images negative in relief to the previously described etch-out process, and the matrices would therefore be obtained from images negative to, i. e., printed from, that specified for 10 the etch-out process.

While I prefer to use double coated or duplitized positive stock, my process is readily adapted to use a film having one extra thick emulsion only, or two emulsion layers on the same side of the 15 support. The only variation in my process as applied to this type of film is in the first step; namely, the production of the initial two-color print. One method of securing a satisfactory two-color print on such film is to print both 20 negatives as before, one to the face of the positive stock and one through the base to the inside of the emulsion. After developing and fixing both images, the film can then be immersed in a bleaching solution such as an iodide bleach or 25 ferricyanide bleach and left until the outer image has been completely bleached. The film is removed before the inner image is affected and the excess bleach is washed out. The film may then be immersed in a solution of basic dye which will 30 mordant to the bleached image but will not affect the inner image. After this step the film is subjected to a toning solution of a color substantially complementary to the dye previously used, which tones the inner image the desired color without 35 affecting the previously dyed image.

Another way to produce the two-color print on this type of stock is to immerse the film with the developed image in a solution of iron tone until the outer image is fully converted to a blue 40 color and then to quickly remove the film and wash out the excess blue tone to keep it from affecting the inner image. The film can then be immersed in a uranium toning solution to color the inner image red, the uranium tone not affecting 45 the previously iron-toned outer image.

When in the foregoing I use the term three-color as applied to a process or print, it is to be understood that I mean a process employing three-colors in its operation, or a print secured 50 by such a process, and I do not mean to imply that the print reproduces but three colors, for it is well known that by the proper combination of three primary colors, all colors of the visible 55 spectrum can be obtained.

Also, when in the claims I use the phrase "superposed emulsions" it is to be understood that I include emulsions with and without a separating layer between them.

From the foregoing it will be seen that I have 60 developed a process of great simplicity and flexibility for the economical production of three-color photographs from only two color-separation negatives. While the forms of my invention herein described are fully capable of attaining 65 the objects and providing the advantages previously mentioned, I realize that many modifications and variations will occur to those skilled in the art, and it is to be understood that the foregoing description is meant to be merely illustrative of the fundamental principles involved and in no wise as limiting the proper scope of my invention as defined by the appended claims.

I claim as my invention:

1. The method of producing a photograph in color which includes: producing two substantially complementary color-value images in superposed emulsion layers; coloring said images red and blue respectively; and imbibing a yellow dye image of the green to red color values of the same subject on top of one of said first mentioned images.
2. The method of producing a photograph in color which includes: producing a blue to green color-value negative and a green to red color-value negative; producing positive images from said negatives in superposed emulsion layers; coloring the positive image produced from the green to red color value negative blue; coloring the positive image produced from the blue to green negative red; producing from one of said negatives a matrix having a green to red color value relief image; applying a yellow dye to said matrix; and imbibing a yellow image on one of said positive images by means of said matrix.
3. The method of producing a photograph in color which includes: photographically producing blue to green and green to red color-value positive images in superposed emulsions; treating said images to give them a blue and red color respectively; and imbibing a third image on one of said emulsions by means of a relief image matrix having a green to red color value image of the same subject carrying a yellow dye.
4. The method of producing a photograph in color which includes: producing blue to green and green to red color-value images in separate emulsion layers on opposite sides of a support; toning said first image blue; coloring said second image red; and imbibing a third image on one of said emulsions by impressing thereon a matrix having a green to red color value image of the same subject carrying a yellow dye.
5. The step in a three-color photographic process which includes: making a matrix for use therein, by producing two substantially complementary color-value negatives; making a combined print of said negatives; making a separate print of one of said negatives; superposing on said separate print a print from said combined print; developing and fixing said superposed printed images; and treating said film to remove the silver images and the contiguous gelatin therefrom to give a gelatin relief image.
6. The method of making a matrix for use in a three-color process of photography which includes: producing a blue to green color value negative and a green to red color value negative; printing said negatives to opposite sides of a double coated film to give corresponding positive images; making a positive image from the green to red negative only; superposing on said image an image printed from said double coated film; developing and fixing said superposed images; and treating said images to remove the silver and the contiguous gelatin therefrom to give a gelatin relief image.

DONALD K. ALLISON.